

# UNITED STATES PATENT OFFICE.

SIGVALD ALFRED CHRISTIAN KRISTENSEN, OF SÖTORP PER VALBY, NEAR COPENHAGEN, DENMARK, ASSIGNOR TO ANDELSSELSKABET INTERNATIONAL METALLOTYPEKOMPAGNI, LIMITED, OF COPENHAGEN, DENMARK:

## PROCESS OF STEREOTYPING.

No. 840,775.

Specification of Letters Patent.

Patented Jan. 8, 1907.

Application filed July 27, 1905. Serial No. 271,537.

*To all whom it may concern:*

Be it known that I, SIGVALD ALFRED CHRISTIAN KRISTENSEN, stereotyper, a subject of the King of Denmark, residing at Sötorp per Valby, near Copenhagen, Denmark, have invented a certain new and useful Process of Stereotyping, of which the following is a specification.

This invention relates to the production of matrices for the stereotyping of type-forms, line-etchings, and half-tone blocks or the like; and it has for its main purpose to increase the clearness and sharpness of the matrices and their durability and make them better adapted than are the matrices heretofore used to resist the action of several castings, even at higher temperatures than have heretofore been employed.

Up to the present time the casting of stereotype-plates in ordinary paper matrices has been made at temperatures ranging from 280° to 340° Fahrenheit, as the common paper matrices are not able to resist higher temperatures. Alloys of such low melting-points suffer, however, from the defect of being rather soft, a circumstance making it necessary very often to give the stereotype-plates an aftertreatment—nickel and copper plating them, for instance—in order to increase the hardness of their surface, and thus enable them to better resist the pressure and wear caused by the printing; but even when employing such rather low temperatures of casting the ordinary paper matrices cannot be used for more than a very few castings, (in the reproduction of type-forms perhaps two or three,) the reason being that the repeated application of molten metal to the paper matrix makes its surface brittle and burned.

This drawback is especially prominent in the casting of stereotype-plates for rotary presses, because the amount of metal used, and consequently also the quantity of heat contained in such metal, is here very considerable. Ordinary paper matrices are, besides, not very suitable for the stereotyping of fine-line etchings, and they are especially unfit for stereotyping autotypes or so-called "half-tone" etchings, the reason being that the matrix must be made very wet in order to penetrate into the very fine cavities of the form; but consequently when the matrix is dried it will shrink very considerably, and the reproduc-

tion subsequently cast therein will therefore be lacking in accuracy and depth, so that the intaglio cavities between the grains or lines may blacken the prints produced from the stereotype-plate. Ordinary paper matrices suffer, finally, from the defect that they will not at all slip the stereotype-plate founded therein unless they are previously rubbed by graphite, powdered soapstone, or the like, which treatment will of course be detrimental to their sharpness.

The present invention has for its purpose to produce matrices with such a coating on their surface that the matrix is on that account enabled (1) to endure a considerable number of castings; (2) to resist a temperature of casting considerably higher than what has been used heretofore, so that alloys of greater hardness may be employed; (3) to withstand bending without any danger of breaks or cracks in the surface; (4) to take very accurate impressions of the very finest as well as of the coarsest cavities and projections; (5) to be used as a mold without any kind of aftertreatment, such as powdering, greasing, &c.

The solution of the special problem embodied in requirement No. 4 in the above enumeration—namely, on an ordinary paper matrix suitable for stereotyping of type-forms to produce also the very finest impressions—has been attempted by giving those parts of the mixed form (types and half-tone blocks) that have the fine cavities—viz., the half-tone blocks—a coating consisting of whiting or powdered clay, mixed, if desired, with water, which coating is then by wiping removed from the printing-face before the ordinary paper flong is laid on and then treated in the usual way. The paper flong during the treatment is pressed down into the coarse cavities, and thus receives direct imprint of these, while on the fine-cavity parts of the form coated with clay or the like the impression is produced by means of the fine-grained substance that fills the fine cavities of the form and when the wet paper flong is laid on under pressure adheres to the flong and stands out from its surface after it is removed from the form. Even admitting that an impression of the fine relief of the form may be made in this manner, it is nevertheless not deep or sharp enough to give a fault-

less reproduction of the original in such a matrix. This drawback is due partly to the fact that the substances used will shrink considerably during the subsequent drying, and 5 consequently be subject to the formation of fissures and crevices, and partly to the circumstance that the air lodged in the cavities of the autotype cannot escape when a paste such as the one above described is applied to 10 the autotype, and consequently will prevent the paste from penetrating to the very bottom of the cavities and from closely following their sides. For these reasons the relief becomes inaccurate and full of fissures and 15 also too low. Printing-plates cast in such a matrix will therefore be liable to blacken the prints taken therefrom and generally will not give as sharp and clean prints as the original. The matrices produced in the above-de- 20 scribed manner will further suffer from other defects and drawbacks, some of which are to be mentioned in the following: The impression-surface is very easily fractured, because chalk, clay, and the like are brittle sub- 25 stances, the grains of which are liable to break when the matrix is bent, or even when it is removed from the form after drying. Besides, it is liable to be damaged if touched. These substances are also porous, and during 30 their drying fissures have arisen. They will therefore not easily slip the cast metal, and as they are brittle it happens often that the grains break off when the matrix is removed and remain in the cavities of the original 35 etching. This is unfortunate, partly on account of the damage to the matrix and partly because the etching has to be carefully cleaned before it can be used again. This cleaning is exceedingly difficult and can, in 40 fact, only be made by chemical means; but the adhering chalk, &c., can only be dissolved by using acids, and the latter will also very rapidly attack the etching itself, especially if it is a zinc etching, and very likely 45 destroy it completely. Finally, it may be mentioned that the substances used are bad conductors of heat, so that the matrices become brittle and burned when the metal is cast therein and will endure only a very few cast- 50 ings, even at low temperatures.

According to the present invention the entire face of the matrix is coated with a metallic film, endowing it with all the desirable qualities enumerated before under 55 headings 1-5, and the substances as well as the process employed for this purpose insure that the matrix thus obtained will become an exact negative copy of the relief of the form.

60 The substance to be applied to the form consists, according to the present invention, of a liquid mixture of finely powdered or pul- 65 verized metal. Such mixture may be formed of about ten per cent. of borax in water, to

bring the mass to a pulpy condition, after which a volatile medium, such as alcohol, is added to bring the mass to a liquid state. A sufficient quantity of the powdered metal may then be added.

Especially aluminium powder is eminently suitable as a metal for the purpose mentioned, partly because it is easily held in suspension in the proper amount of liquid and partly because it may in contrast to the substances heretofore used easily and quickly be dissolved by a weak solution of sodium hydrate, which practically will not attack the zinc, so that even if by inadvertence a part of the metallic skin might remain in and on a 80 zinc etching the latter could be easily washed free of such remnants without damage to itself.

The method of producing such a matrix coated by metal is preferably as follows: The 85 form (type matter, etchings, galvanoes, wood, cuts, and the like, or mixtures of these) after being slightly greased is coated by the above-described liquid. Thus all the cavities of the form are filled by a metallic powder, and over 90 the entire face of the form remains after drying a continuous metallic form. On top of this is placed, in the usual way, the damp paper flong, and the whole thing is then treated in the matrix-press according to the ordinary 95 method used in the so-called "hot" stereotyping. The metallic film on the form is thus transferred to the surface of the matrix, so that when the matrix is removed from the form the film too leaves the form and adheres 100 to the matrix, forming on its face a continuous metallic film or skin presenting an exceedingly fine and accurate negative reproduction of the form.

The great and general superiority of this 105 process over the methods formerly employed is mainly due to the employment of a metallic powder as the filling mass. The reason is that in drying this will not shrink appreciably, and in consequence the imprint on 110 the matrix will be just as sharp and deep as the relief of the form itself. The metallic film on account of being both hard and still somewhat elastic is also highly tenacious, both against bending of the matrix and 115 against casual handling and wear. It is, further, proof against even much higher temperatures than those used in stereotyping and has a high heat-conducting power. By this circumstance is attained the advantage of being 120 able to use in the casting alloys of higher melting-point, and therefore greater hardness, than those usually employed, whereby the necessity of subsequently hardening the face of the stereotype-plate, as described before, is 125 avoided, and, besides, the heat in the metal poured in is evenly distributed over the whole paper mass below, so that this is well protected and does not become brittle, or even burned. Finally, the metallic particles are not porous, 130

and in consequence the metal poured out on the metallic skin will after solidifying very easily slip the matrix, there being no necessity for greasing the latter, whereby its sharpness would be diminished before making the casting. Another very essential feature of the invention is the employment of the substance in a liquid state, whereby the metal powder is allowed to settle, so as to form a solid film closely following the finest cavities of the autotype.

In the claims I have used the term "printing-form" to include all kinds of type matter, galvanoes, etchings, half-tone etchings, and the like, the invention being perhaps of greatest importance in connection with half-tone etchings.

Having now particularly described and ascertained the nature of my said invention and 20 in what manner the same is to be performed, I declare that what I do claim is—

1. The process for making matrices for a stereotype from a printing-form, which consists in coating such form with a volatile fluid 25 containing an adhesive substance and a metallic powder, and after drying forming a matrix or flong of paper or papier-mâché thereon, said coating being transferred to the said matrix and forming when the matrix is dried 30 a continuous and tough metallic film or skin extending over the face thereof.

2. In the making of matrices for a stereotype wherein a flong of fibrous material is pressed onto the printing-form, the process which consists in coating one of said devices 35 with a liquid containing a fine metallic powder, and then pressing the flong and form together to form the matrix, such coating constituting a part of the matrix when the latter is removed, and forming a metallic film or 40 skin extending over the face thereof.

3. In the making of matrices for a stereotype wherein a flong of fibrous material is pressed onto the printing-form, the process which consists in coating one of said devices 45 with a liquid containing a fine aluminium powder, and then pressing the flong and form together to form the matrix, such coating constituting a part of the matrix when the latter is removed, and forming a metallic 50 film or skin extending over the face thereof.

4. A paper or papier-mâché matrix for stereotyping a printing-form, having on its face a dry and solid film consisting of a metallic powder with an adhesive as a carrier. 55

In witness whereof I have hereunto set my hand in presence of two witnesses.

SIGVALD ALFRED CHRISTIAN KRISTENSEN.

Witnesses:

JULIUS SELEMANN,  
ALBERT G. MICHELSSEN.